

1

3,211,819

PROCESS FOR THE PRODUCTION OF TIRES OF  
SMALL DIMENSIONS

Raymond Guyot, Paris, France, assignor to Textile & Chemical Research Company (Vaduz) Limited, a corporation of Liechtenstein

No Drawing. Filed Mar. 26, 1963, Ser. No. 267,915

Claims priority, application France, Mar. 29, 1962,  
892,693

1 Claim. (Cl. 264—326)

This invention relates to the production of pneumatic tires, and relates more particularly to the preparation of pneumatic tires of small dimensions reinforced by cabled yarns of synthetic materials.

Cabled yarns consisting of synthetic textile materials, notably those based on polyamides such as polyhexamethylene adipamide, are being employed on an increasing scale in the reinforcement of pneumatic tires. In the case of tires of large calibre, it has proved necessary to subject the prevulcanized articles to an expansion in order to compensate for the shrinkage which cabled yarns consisting of synthetic textile fibres undergo at the vulcanization temperature.

However, expansion is impractical in the case of tires for bicycles for reasons of cost. In small-size tires for this application, cabled yarns of synthetic textile fibres have interesting advantages such as high tensile strength, low sensitivity to water and impact resistance.

The manufacture of small-size pneumatic tires without expansion has given rise to serious disadvantages, of which the two main ones are:

(1) The cabled yarns tend to protrude into the interior of the tires.

(2) The tires are often greatly deformed and twisted.

These two defects are due to the shrinkage of cabled yarns at the vulcanization temperature.

According to the present invention, these defects can be obviated and pneumatic tires reinforced with cabled yarns consisting of synthetic textile materials having entirely satisfactory appearance and properties can be produced without the aid of expansion after the prevulcanization by use of rubber preparations having a high rate of vulcanization, the rubber which envelopes the cabled yarns of synthetic textile fibres having to reach a sufficient consistency before the cabled yarns can contract due to thermal action.

For cabled yarns consisting of polyhexamethylene adipamide, use is made more especially of preparations which have a vulcanization rate corresponding to 3 minutes or less, measured on the Wallace vulcanometer, at a vulcanization temperature of 140° C.

The invention is illustrated by the following example of an embodiment, but it is to be understood that this example has no limiting character and that the invention also includes any variant in the same spirit.

2

*Example*

Cabled yarns, 420/2, consisting of polyhexamethylene adipamide with a twist setting of 600 Z-600 S are subjected to a combined overstretching and setting at elevated temperature corresponding, for example, to an increase in length of 8%.

The adhesion treatment of the cabled yarns may be combined, if necessary, with the overstretch with setting. The cabled yarns obtained are calendered in the form of sheets without stentering or in the form of previously stentered sheets.

The following rubber mix is suitable for the calendering of these sheets, the parts being by weight:

|    |                        |     |
|----|------------------------|-----|
| 15 | Natural rubber         | 110 |
|    | Synthetic rubber "SBR" | 90  |
|    | Carbon black           | 55  |
|    | Inert mineral filler   | 105 |
|    | Mineral oil            | 8.5 |
| 20 | Diphenylguanidine      | 0.9 |
|    | Mercaptobenzothiazole  | 1.6 |
|    | Zinc oxide             | 8.5 |
|    | Sulphur                | 4   |

The calendered sheet is molded and it is vulcanized for 3 minutes at 185° C. The tires removed from the mold are free from the aforesaid defects and have entirely satisfactory appearance and properties.

It is to be understood that the foregoing detailed description is given merely by way of illustration and that many variations may be made therein without departing from the spirit of this invention.

What is hereby claimed and desired to be secured by Letters Patent is:

The process for the production of small size tires for bicycles which are reinforced by nylon tire cords, capable of undergoing shrinkage under the action of heat as used during vulcanization, which comprises embedding said nylon tire cord reinforcement in a rubber mix which is capable of being vulcanized in three minutes at a temperature of 140° C. molding and vulcanizing said mix at said temperature under conditions to produce a tire wherein the nylon cords have not been appreciably shrunken.

45

References Cited by the Examiner

UNITED STATES PATENTS

2,623,024 12/52 Barton ----- 260—5  
2,679,088 5/54 Meherg et al. ----- 152—359

50

FOREIGN PATENTS

597,556 1/48 Great Britain.

OTHER REFERENCES

Introduction To Rubber Technology, edited by Maurice 55 Morton, copyright 1959, pages 100 and 101 relied upon.

ARTHUR L. LA POINT, Primary Examiner.